

July 2, 1929.

E. GATHMANN

1,719,544

METHOD OF MAKING INGOT MOLDS

Original Filed Sept. 15, 1926 2 Sheets-Sheet 1

Fig. 1.



Fig. 3.



Fig. 2.



Fig. 4.



Fig. 5.



Emil Gathmann, Inventor

By

Paulson Wright

Attorneys

July 2, 1929.

E. GATHMANN

1,719,544

METHOD OF MAKING INGOT MOLDS

Original Filed Sept. 15, 1926 2 Sheets-Sheet 2



Emil Gathmann, Inventor  
by their Attorneys.

Right

Patented July 2, 1929.

1,719,544

# UNITED STATES PATENT OFFICE.

EMIL GATHMANN, OF BALTIMORE, MARYLAND.

## METHOD OF MAKING INGOT MOLDS.

Original application filed September 15, 1926, Serial No. 135,586. Divided and this application filed October 8, 1928. Serial No. 311,203.

This application is a division of my application for patent No. 135,586, filed September 15, 1926, which contains claims to an ingot mold having the characteristics shown 5 in the accompanying drawings and herein-after described.

This invention relates to metallic ingot molds of the class having vertical ingot-forming chambers and particularly to molds 10 which are open at top and bottom with walls relatively thick in their lower portion and gradually decreasing in thickness upwards. In pouring or teeming such molds the stream of highly heated molten metal, in 15 the first part of the pouring, strikes the mold chamber walls in the lower portion of the mold chamber with great force and heretofore has often cut into the mold walls and suddenly heated them, thereby setting up 20 strains or stresses which cause cracks or recesses to be formed which often seriously impair the life or efficiency of the mold and make the stripping operation difficult.

The object of my present invention is to 25 prevent the formation of such cracks or recesses and to thus lengthen the life of the mold and to facilitate the stripping operation.

Broadly stated, my invention consists in 30 rendering harder and more heat resisting the lower portion of the inner walls of the mold chamber than the mold walls above such lower portion so that said lower walls may receive the impact of the stream of 35 molten metal without being injured while the upper walls retain the desirable characteristics of the cast iron usually employed in making ingot molds.

The accompanying drawings are largely 40 diagrammatic, but sufficiently illustrate the best ways now known to me of carrying out my invention.

Figure 1 shows a vertical section of an 45 ingot mold of well known construction with my improvements applied.

Figure 2 is a sectional view of the lower portion of the mold, the section being taken on the line 2—2 of Figure 1.

Figure 3 shows a vertical section of an 50 ingot mold provided with a modified form of my invention.

Figure 4 is a sectional view of the lower portion of the mold, the section being taken on the line 4—4 of Figure 3.

Figure 5 is a view similar to Figure 4, the

section being taken on the line 5—5 of Figure 3.

Fig. 6 is a central, vertical sectional view of a sand forming mold used for casting an ingot mold embodying one form of my invention.

Fig. 7 is a view similar to Figure 6 and showing a sand forming mold used for casting an ingot mold embodying another form of my invention.

I will first describe the characteristics of the molds shown in the drawings and will then describe the method of making them.

The mold shown in Figure 1 has an ingot forming chamber A larger in diameter or 70 cross section in its upper than in its lower portion, the chamber gradually or progressively increasing in width from bottom upwards. The mold is open at top and at bottom and the lower portion of the mold chamber is necked-in by inner mold walls a having a concavo-convex contour of the kind shown, described, and claimed in my U. S. Patent No. 1,188,751, of June 27, 1916. The bottom opening B of the mold may be closed 80 by a plug C in the usual way or by other suitable means. The walls of the mold are thicker in their lower portion than in their upper part for a purpose now well understood and the mold, for the most part, is 85 made of cast iron of the usual kind. Generally such molds are made of an open grade of bessemer cast iron containing approximately the following ingredients: silicon 1.25; manganese 0.80; sulphur (under) 0.06; 90 phosphorus (under) 0.20; total carbon 3.75. The contained graphitic carbon usually runs from 3% to 3½%. Cast iron, having these characteristics being of a so-called open structure, admirably fulfills an important 95 requirement in ingot molds, viz: It has the capacity of expanding and contracting correspondingly with the variations in temperature incident to the formation of ingots in the mold chamber without fracturing of the 100 mold walls or excessive cracking. But the melting point of such cast iron or mold metal (2,200° F. to 2,300° F.) is relatively low compared with the temperature of steel while being cast, which varies from 2,600° 105 F. to 2,900° F. and at times is even higher.

As a highly heated stream of molten metal enters a mold chamber and strikes against the bottom or lower walls of the chamber, which at first are relatively cool, it often 110

cuts, erodes, or even melts the mold walls with which it comes in contact, or so heats said walls as to cause such strains or stresses to be produced as will cause cracks or recesses therein. This has often so changed the contour of the lower portion of the mold chamber as to render the mold inefficient and this has often occurred long before the upper portion of the mold has been seriously impaired. This wearing away of the mold walls is primarily due to cumulative strains produced by continued expansion and contraction of the mold walls caused by temperature changes.

15 If an ingot mold were made entirely of steel, which has a high melting point and hence greater heat resisting qualities than cast iron, the mold walls would be more resistant to the cutting and erosive action of the liquid steel poured into the mold, but steel walls are not suitable for making ingot molds because such steel walls do not so readily expand and contract as do mold walls made of cast iron, and therefore they would warp to such an extent as to prevent the removal of the ingot from the mold. Furthermore, the cost of steel molds would be so much greater than cast iron molds that steel could not be used economically. I therefore make the mold principally of cast iron as heretofore and so form or so treat the lower portion of the inner mold walls as to render them harder and more heat resisting than the remaining walls. This may be accomplished in various ways. One way is to form the lower inner mold walls of an alloy of iron with a substance having a high melting point, such as vanadium, molybdenum, tungsten, chrome, or other such metal.

20 Vanadium, for instance, has a melting temperature of approximately 3100° F., which is considerably higher than the temperature of steel when teemed into a mold.

25 It will be understood that the lower portion only of the mold walls should be given the heat resisting qualities above mentioned in order that the upper part of the walls shall have the desirable characteristics of expanding and contracting without cracking, which, as before stated, is inherent in gray iron of the kind generally employed in making ingot molds.

30 Ingot molds of the kind shown are usually cast in sand flasks, bottom end uppermost.

35 Fig. 6 illustrates a forming mold set up which may be used for producing an ingot mold provided at its lower chamber portion with a block of heat resisting material according to my invention. The mold set-up includes the usual flask H, sand I rammed therein, a sand core J supported upon a metal plate K and positioned centrally within the mold cavity, and a sprue L through

40 which molten iron is introduced into the mold cavity. In preparing the flask to cast molds of the kind shown in Figures 1 and 2 with my improvements applied, the core J of the sand mold shown in Fig. 6 is formed in the usual way and a block D of high heat 70 resisting material or having its inner surface provided with heat resisting material is placed on the core at its upper end so that the molten metal will surround the block when it rises in the flask and will be 75 firmly united therewith when the metal cools and solidifies. The block thus constitutes the upper end of the core during the casting operation. Preferably the block D of high heat resisting material or having its 80 inner surface provided with heat resisting material is of the form shown in Figures 1 and 6, being tapered as shown and having a serrated upper edge whereby it may be firmly locked to the main mold walls. In the construction shown in Figure 1, the bottom of the mold chamber is formed in the block D and the necked-in portion of the mold chamber is formed in this block. The block may be formed of an iron alloy of the 85 kind previously described and is, of course, made separately and placed in the same mold in the manner above explained. The block D in the completed mold is not separable from the mold; it is a permanent part there- 90 of.

95 The mold shown in Figures 3, 4, and 5 has the lower walls of the cast-iron mold treated to render these walls highly heat resisting. To accomplish this result, the loam or foundry sand composing that portion of the core for forming the lower part of the mold chamber is impregnated or coated with a flour-like metallic dust adapted to alloy with molten iron when brought into contact therewith such as powdered vanadium, molybdenum, chrome, and the like made into a paste with molasses and water or other such binder. The sand forming mold and core 100 J are then set up as shown in Figure 7 and molten metal introduced into the mold cavity through the sprue L. When the molten metal rises in the sand flask and surrounds the treated core, this treated part of the core or a part thereof adheres to or is absorbed by the cast metal. In this way a lining or a casing of high heat resisting iron or iron alloy is provided in the lower portion of the mold chamber. In Figures 3, 105 4, and 5 the lining or treated portion of the mold wall is indicated at E. The high heat resisting material should not extend to any considerable extent above the necked-in part of the mold chamber as the desired qualities of ready expansion and contraction of the mold would be impaired if any considerable portion of the walls above the necked-in portion were materially changed. While I have shown in the drawings two practical ways of 110 embodying my invention in ingot molds, it 115

120

125

130

will be understood that the details illustrated and described may be varied without departing from the novel features of my invention.

5 The forming molds in which the ingot molds are cast are of usual construction except as modified in the manner above described.

I claim as my invention:

10 1. The herein described method of forming an ingot mold which consists in treating the upper end only of the core of a forming mold with a metallic material which is adapted to alloy with molten iron when brought into contact therewith, and which is highly heat-resisting to the cutting action of liquid steel, and then pouring the ingot mold metal into said forming mold and around said core whereby heat-resisting material on 20 said core will be transferred to that portion of the ingot mold which forms the lower portion of the ingot mold chamber.

25 2. The herein described method of forming an ingot mold which consists in providing the upper curved necked-in portion only of the core of the forming mold with metallic alloying material which is adapted to alloy with molten iron when brought into contact therewith and which is highly heat 30 resistant to the cutting action of liquid steel, and then pouring the ingot mold metal into said forming mold, whereby said metal will combine with the heat resisting material placed on said curved necked-in portion of the core thus forming the inner walls of the 35 lower portion of the ingot mold chamber

of an alloyed more heat-resisting to the cutting action of liquid steel than the upper portion of said mold walls.

3. The method herein-before described of 40 producing an ingot mold which consists in forming a core of a forming mold of suitable material, treating the upper portion only of said core with a finely divided alloying material which is adapted to alloy with 45 molten iron when brought into contact therewith and which is of high melting point, and then pouring the ingot mold metal into the forming mold and around the core whereby said alloying material will be transferred 50 to said mold thus rendering the lower chamber portion only of the resulting ingot mold more highly resistant to the cutting action of liquid steel cast therein than the remainder of the mold. 55

4. The herein-described method of forming an ingot mold which consists in placing upon that end portion of the core of the forming mold which is to form the lower matrix wall of the ingot mold, metallic material 60 adapted to unite with molten iron when brought into contact therewith, and which is more heat resisting to the cutting action of liquid steel than the ingot mold metal, and then pouring the ingot mold metal into 65 the forming mold and around the core whereby said material is united with the ingot mold at the lower chamber portion thereof.

In testimony whereof, I have hereunto subscribed my name.

EMIL GATHMANN.